

Dec. 27, 1932.

B. STOCKFLETH

1,892,173

METHOD OF MAKING THIN WALLED METAL ARTICLES

Filed Feb. 11, 1929

2 Sheets-Sheet 1



Witness: 5 10 8

Harry R. White

Inventor:  
Berger Stockfleth  
By Edward Fay Wilson  
Dec.

Dec. 27, 1932.

B. STOCKFLETH

1,892,173

METHOD OF MAKING THIN WALLED METAL ARTICLES

Filed Feb. 11, 1929

2 Sheets-Sheet 2

FIG. 2.



FIG. 3.



FIG. 4.



FIG. 5.



FIG. 6.



Witnesses:

Harry R. White 10

Edward Hay Wilson 15

Inventor:

Berger Stockfleth

Edward Hay Wilson  
duly

## UNITED STATES PATENT OFFICE

BERGER STOCKFLETH, OF NILES, MICHIGAN, ASSIGNOR, BY MESNE ASSIGNMENTS, TO THE CLEVELAND GRAPHITE BRONZE COMPANY, OF CLEVELAND, OHIO, A CORPORATION OF OHIO

## METHOD OF MAKING THIN WALLED METAL ARTICLES

Application filed February 11, 1929. Serial No. 339,170.

This invention relates to improvements in renewable bearing sleeves and their manufacture and especially to such bearings as have backings of relatively hard metal and 5 linings of relatively softer bearing metal.

In my earlier co-pending application, filed August 20, 1928, Serial No. 300,757, which matured into Patent No. 1,803,513, issued May 5, 1931, I have shown a bearing 10 of the kind mentioned, having a formed-up sheet steel back and a Babbitt metal lining, and said co-pending application shows a novel method of making such a bearing.

I have found that the formed-up sheet steel 15 blanks for the backs are more or less wavy; that is, they are not exactly true. This results from the process of manufacture with the usual or ordinary forming-up dies and presses. On the other hand, the sleeves 20 when finished must be exactly true within certain very small tolerances, and by means of my present invention I am enabled to produce the sleeves to dimensions and form as close to the desired dimensions as is called 25 for under the more recent requirements of rapid production manufacturing developments.

Another important feature of this present invention is that it results in a better adherence 30 of the Babbitt metal lining to the backing, particularly adjacent to the longitudinal edges of the bearing shell. This is accomplished by allowing the backing to be elongated circumferentially with the Babbitt 35 metal lining in the pressure forming step instead of hindering such elongation of the backing as heretofore. In this present invention, I permit both the Babbitt metal lining and the backing to be extruded from the 40 dies, under the heavy forming pressure, along the longitudinal edges of the shell and thus do not disrupt the bond between these two layers.

Furthermore, as the backing is allowed to 45 elongate circumferentially, the waves or irregularities are smoothed out in such movement between the inner and outer surfaces of the dies in what is aptly termed an "ironing-out process." I find that I am enabled to 50 form the bearing shells with less pressure

than formerly, to make them more accurate and better, and to make them quicker, all of which is of great value when we consider the quantity production which is necessary.

A particularly valuable feature of this 55 present invention relates to the production of bearing sleeves having external end flanges.

For the purpose of producing the bearing sleeves rapidly and accurately and in large 60 quantities, the backs or shells are formed up out of sheet metal and the end flanges thus formed are quite irregular in shape, it being necessary that the metal be upset or stretched 65 in order to produce these end flanges.

By means of this present invention, these 70 end flanges, as well as the body or cylindrical part of the shell, are ironed out smooth, the resultant bearing sleeve having accurately dimensioned and smooth end flanges. This 75 is accomplished by allowing the end flanges as well as the body portion to be elongated circumferentially under the tremendous pressures used and held against enlargement in other directions, at some points being 80 thinned as to thickness.

The invention will be more readily understood by reference to the accompanying drawings forming part of this specification and in which—

Fig. 1 is a perspective view of a finished half cylindrical bearing sleeve having end flanges and made in accordance with this invention;

Fig. 2 is a fragmentary perspective view 85 of a flanged backing shell, showing it as it appears when first formed, the irregularities or waves being greatly exaggerated;

Fig. 3 is a developed section of the flange on the line 3—3 of Fig. 2;

Fig. 4 is a sectional view of a press, taken 90 on the line 4—4 of Fig. 5 and showing the press forming a flanged bearing;

Fig. 5 is a fragmentary vertical section on the line 5—5 of Fig. 4;

Fig. 6 is a fragmentary horizontal section 95 on the line 6—6 of Fig. 4;

Fig. 7 is a cross-sectional view of a sleeve back without flanges as it appears when first 100 formed up;

Fig. 8 is a view similar to Fig. 7, showing the backing after having been coated with the bonding metal;

Fig. 9 is a similar view with the addition 5 of the lining of bearing metal;

Fig. 10 is a sectional view of a press similar to Fig. 4, showing the sleeve, as shown in Fig. 9, in place in the dies ready to be finished; and

10 Fig. 11 is a similar view of the press showing the sleeve at the end of the pressing operation.

In said drawings, 1 indicates a finished half cylindrical bearing sleeve. This consists of an outer relatively harder backing shell 2, preferably made of steel or bronze, and an inner lining 3 of bearing metal such as babbitt. The Babbitt metal is bonded to the backing by a coating 4 of tin between them, and the outer surface of the backing 2 is coated with the bonding metal as shown at 5. It should be understood that the thickness of the various parts is more or less exaggerated. This applies especially to the tin coating.

As shown in the drawings, the bearing sleeve has external end flanges 6 which, like the body, are composite; that is, the steel shell 2 has end flanges 7 which form the backs 30 or inner parts of the flanges 6, and the outer surfaces 8 of the completed flanges 6 are formed of the Babbitt metal similar to the structure of the body of the sleeve. For some purposes, the bearing sleeves are not provided with the flanges 6, and in Figs. 8 and 9 the formation of such sleeves is illustrated.

In the production of the sleeves, the backing 2 is first formed up, preferably out of sheet metal, and in this process, using the 40 ordinary forming-up presses, these backings are more or less irregular in shape; that is, they are not accurate as to size or shape. This irregularity is indicated by the more or less wavy outlines, as indicated at 2.

45 The backing thus formed is next dipped in a molten bonding metal such as tin and is thus given the coating of tin, as shown at 8 and 9. The next step is to add the inner lining 3 of bearing metal, and this is preferably done in 50 accordance with my invention as described in my co-pending application filed August 20, 1928, Serial No. 300,757, entitled "Means and methods for making bearing linings or sleeves"; that is, by casting the lining onto 55 the inner surface of the backing, the tin coating on said inner surface being effective to cause the bonding of the bearing metal lining to the backing. The backing 2 is still in its condition as first formed up; that is, it is 60 irregular as to shape and not accurate as to dimensions.

The next step is to form and size the bearing sleeve. This is accomplished in a pair of die members 8 and 9. The lower die member 65 8 has a half cylindrical opening 10 for receiv-

ing and shaping the outer surface of the bearing sleeve, and the upper member 9, which is the plunger, has a lower half cylindrical end 11 adapted to cooperate with the die member 8 and shape and form the inner surface of the bearing shell. 70

Means, not shown, are provided to close the ends of the opening 10 and to limit the closing of the dies together to accurately size the bearing sleeves. 75

The pressing operation, as illustrated in Figs. 10 and 11, requires a tremendous pressure, and under the heavy pressure the backing 2 as well as the lining 3 are elongated circumferentially, being actually forced out 80 or exuded from the die space as indicated at 12, Fig. 11.

This present invention is useful particularly in quantity production, and the allowable tolerance is very small, hence any change 85 in the dies is fatal to the accuracy of the production. As the relatively hard back is elongated, as described, and as this elongation takes place under such heavy pressure, the wear—particularly on the lower die 8—would 90 be very great and would soon destroy its usefulness if it were not for the outer coating 5 of the tin. This coating, being of a relatively soft and malleable metal, serves as a lubricant between the die surface and the backing 95 shell and permits the elongation of the backing shell without any appreciable wear on the die member 8.

The tin on the outer surface of the back 100 removes the necessity for the elimination of all of the irregularities in the backing shell, as the tin coating provides an outer surface which accurately conforms to the forming surface of the die member 8 and tends to fill up any slight depressions which might remain.

The action in the press may be very well described as an "ironing out of the wrinkles or waves." This cannot be done by mere pressure alone but needs the movement of the metal of the backing between the die members at the time of the application of the forming pressure. 110

The process above described applies also to the ironing out of the wrinkles, waves or irregularities in the end flanges 7 of the backing shell. These irregularities are indicated at 13, Figs. 2 and 3.

Figs. 4 to 6, inclusive, illustrate the ironing out process as applied to the end flanges 120 of the bearing sleeve. The sleeve is built up of a back and a lining as before, both of these extending into and forming the end flanges 6. The dies for this purpose are similar to the dies already described, consisting of an upper member 14 and a lower member 15, but are formed to provide circumferential cavities 16 at the ends of the dies in which the flanges 6 are sized. The upper die member 14 has end extensions or flanges 17 which 125

close down over the ends of the lower die member and close the cavities 16. It is obvious that upon the closing of the die members together, the cavities 16 being substantially filled with the rough formed flanges, the metal of the bearing shell will be forced with great pressure into said cavities. The cavities are open at their tops and the flanges are free to be forced up and out of the cavities, as indicated at 18, Fig. 4. In other words, the flanges are elongated by the tremendous pressure to which they are subjected. This pressure not only elongates the flanges circumferentially, thus ironing out the wrinkles, but also compresses and compacts the Babbitt metal forming the outer surfaces of the flanges. As in the case of the body portion, the tin coating on the backs of the flanges assists in this process, permitting the movement of the flanges between the opposed surfaces of the die members without undue friction or wear upon the die members.

It should be understood that the excess or the exuded portions 11 are removed in some suitable manner, as by cutting, in order to completely finish the sleeve as shown in Fig. 1.

I claim:

1. The herein described step in the pressure method of making a substantially semi-cylindrical lined bearing sleeve comprising a tough strong supporting back such as steel and a bearing metal lining bonded thereto, and which consists in applying sufficient pressure to a roughly formed bearing by means of dies having semi-cylindrical co-operating pressure surfaces to cause the metals of the sleeve to be thinned radially and elongated substantially parallel to the die surfaces, thereby causing the waves or irregularities in the backing to be "ironed out".

2. In the pressure method of sizing and finishing a bearing sleeve or shell which consists of a backing of relatively hard metal and a lining of relatively soft bearing metal, the steps of providing a bearing sleeve roughly formed to substantially semi-cylindrical shape, the blank comprising a relatively tough strong back and a bearing metal lining bonded thereto, coating the outer surface of the back with a relatively soft metal such as tin, applying forming pressure to the rough sleeve between suitable die members, the pressure applied being sufficient to thin the back and elongate it circumferentially, the soft metal coating on the back allowing the sleeve to move more readily on the adjacent die member and serving to fill in any irregularities not smoothed out by the applied pressure.

3. In the pressure method of sizing and finishing a bi-metal bearing sleeve or shell having a backing of relatively tough strong metal, such as steel, and which consists in coating a roughly formed back on its outer

surface with a relatively soft metal, placing the shell between die members and applying pressure sufficient to cause the backing to be thinned radially and elongated circumferentially, whereby the irregularities are, at least, partly smoothed out, the coating serving to reduce the friction between the backing and the die member against which it is pressed, and to fill any irregularities not entirely smoothed out and whereby the outer surface of the sleeve is accurately of the shape and size of the contacting die surface.

4. The herein described method of making a flanged composite bearing sleeve of the kind described, which consists in forming up a backing with integral flanges at its ends out of a harder metal from a flat sheet, coating the backing with a bonding metal such as tin, applying a bearing metal such as babbitt to the inner side of the main portion of the backing and the outer surfaces of the flanges, then sizing and finishing the sleeve by pressure applied between suitable die members and causing the irregularities in the backing and flanges to be smoothed out by elongating these parts circumferentially while pressed between the die members.

5. The herein described method of producing a flanged bearing-sleeve back out of sheet metal, which consists in roughly forming a flanged back out of sheet metal, in which condition the flanges are more or less wrinkled, and subjecting the roughly formed back to pressure applied by suitable dies substantially normal to the flanges sufficient to cause the circumferential elongation of the flanges and the flattening out of the wrinkles.

6. The herein described steps in the pressure method of making composite bearing sleeves having end flanges, which consist in providing a backing having integral end flanges of relatively harder metal formed up roughly out of sheet metal, coating the backing and flanges with a bonding metal such as tin, applying a lining of bearing metal such as babbitt to the inner surface of the backing and the outer surfaces of the flanges, and ironing out the irregularities in the flanges by applying sufficient pressure between suitable pressure members to elongate the flanges circumferentially while so pressed, the bonding metal on the backs of the flanges assisting in this elongation.

7. The herein described steps in the pressure method of making lined bearing sleeves which consist in providing a roughly pre-formed sleeve back of relatively harder metal, the back having irregularities, and a lining of bearing metal thereon, both thereof slightly thicker radially than in the finished sleeve, applying sufficient pressure radially between suitable die members to cause both the back and the lining to be thinned radially and substantially equally elongated substantially parallel with the die surfaces while confined

between the die members, and whereby the irregularities in the back are smoothed out.

In witness that I claim the foregoing as my invention, I affix my signature this 18th day  
5 of January, 1929.

BERGER STOCKFLETH.

10

15

20

25

30

35

40

45

50

55

60

65